

J. B. LOMAX,  
FINISHING OR LUSTRING TEXTILE FABRICS.  
APPLICATION FILED APR. 10, 1920.

1,393,296.

Patented Oct. 11, 1921.



INVENTOR:  
Joseph Bolton Lomax  
By Wm Wallace White  
ATTY.

# UNITED STATES PATENT OFFICE.

JOSEPH BOLTON LOMAX, OF FURNESS VALE, NEAR STOCKPORT, ENGLAND.

## FINISHING OR LUSTRING TEXTILE FABRICS.

1,393,296.

Specification of Letters Patent. Patented Oct. 11, 1921.

Application filed April 10, 1920. Serial No. 372,866.

To all whom it may concern:

Be it known that I, JOSEPH BOLTON LOMAX, a subject of the King of Great Britain, residing at Birch Lea, Furness Vale, near Stockport, in the county of Derby, England, have invented new and useful Improvements in Finishing or Lustring Textile Fabrics, of which the following is a specification.

10 My invention relates to an improved and continuous process and apparatus for finishing or lustring textile fabrics such as sateens, batistes and the like, but it is applicable to various other classes of fabrics 15 whether mercerized or unmercerized.

In carrying my invention into effect I pass the fabric through a heavy Schreiner calendering machine on which I use a much heavier pressure, say from two to three times 20 as great as for ordinary Schreinering, and I also employ a greater heat to bring the engraved roller to a blue heat or to as great a heat as the cloth will stand without injury.

Immediately the fabric leaves the nip of 25 the Schreiner calendering rollers and while still heated I pass it under tension in the same machine over or under a rotating roller mounted in a box or receptacle and partially immersed in a finishing liquor contained therein by which a film of the liquor 30 is applied to one side or both sides of the heated fabric.

The accompanying drawing shows in elevation a known form of Schreiner calendering machine which I employ for the purposes of my invention. This machine consists of a frame or pedestal *a* carrying the pair of Schreinering calendering rollers of which the upper roller *b* is engraved and 40 brought to a blue heat or as great a heat as the cloth will stand without injury and the lower roller *c* is carried on a ram *d* of a hydraulic press in the usual way. The fabric *e* to be treated is led from the batch 45 roller *i* through the usual tensioning device *f* between the nip of the rollers *b* and *c* where it is subjected to a pressure from two to three times as great as that employed for ordinary Schreinering. Immediately after 50 leaving the nip of the rollers *b* and *c* a film of finishing liquor contained in a trough *g* and maintained at or about boiling point is applied to the underside of the heated fabric

*e* by means of a finishing roller *h* and the fabric *e* is then wound on an ordinary batch 55 roller *i*, which may be rotated by any suitable means, such for instance as a belt and pulley from any convenient source of power. The fabric is left to stand batched in its wet state for about 10 to 12 hours, and then 60 stretched and dried on an ordinary hot air stentering machine and conditioned after which it is ready for making up in the ordinary way.

In the example shown the heated fabric *e*, 65 which may be either mercerized or unmercerized, is led over the finishing roller *h* and the boiling finishing liquor applied to the underside but it will be readily understood that if required the fabric may be guided 70 under the roller *h* and the finishing liquor applied to both sides. The finishing liquor is composed preferably of a boiling solution of alizarin oil say a 10 to 20 per cent. solution of alizarin oil. 75

By my improved process I obtain a fabric (either mercerized or unmercerized) on which the color is more intensified and with a sheen or luster which will resist rain and weather without spotting and will stand 80 washing in hot or cold water without any deterioration after drying.

What I claim as my invention and desire to secure by Letters Patent of the United States is:—

1. The process of finishing textile fabrics which consists in passing the same between a plurality of rollers under high pressure and heat and while hot applying thereto a boiling finishing liquor while retaining the fabric under tension, and winding said fabric into a roll while in hot condition. 85

2. The process of finishing textile fabrics which consists in passing the same between a plurality of rollers under high pressure 95 and heat and while hot applying thereto a boiling solution of alizarin oil while retaining the fabric under tension, and winding said fabric into a roll while in hot condition.

3. In a machine for finishing textile fabrics, 100 the combination with a calendering machine having a pair of calendering rollers, a pair of batch rollers one at each side of said calendering rollers, and tensioning means, of a receptacle for a boiling finishing liquor located adjacent to and parallel with said calendering 105

rollers, and a finishing roller disposed longitudinally partly within said receptacle and having a portion of its circumference in the path of the fabric when passing from the 5 calendering rollers to one of said batch rollers, whereby the finishing roller will take up a portion of the finishing liquor and ap-

ply it to the fabric immediately as the latter emerges from the calendering rollers and while in hot condition.

In testimony whereof I have signed my name to this specification.

JOSEPH BOLTON LOMAX.